

# UNITED STATES PATENT OFFICE.

CLEMENT L. PERKINS, OF PITTSBURGH, PENNSYLVANIA, ASSIGNOR TO METALS RECOVERY COMPANY, OF NEW YORK, N. Y., A CORPORATION OF MAINE.

## FLOTATION OF MINERALS.

1,364,305.

Specification of Letters Patent.

Patented Jan. 4, 1921.

No Drawing.

Application filed July 21, 1919. Serial No. 312,248.

To all whom it may concern:

Be it known that I, CLEMENT L. PERKINS, a citizen of the United States, residing at Pittsburgh, in the county of Allegheny, State of Pennsylvania, have invented certain new and useful Improvements in Flotation of Minerals; and I do hereby declare the following to be a full, clear, and exact description of the invention, such as will enable others skilled in the art to which it appertains to make and use the same.

This invention relates to the concentration of minerals, such as sulfid ores and the like, by flotation, and is based upon the discovery that improved results can be obtained by carrying out the flotation operation with the addition to the ore or mineral pulp of organic nitrogen compounds containing two nitrogen atoms joined to each other, and more particularly azo- or diazo-compounds, such as, for example, diazo-amino-toluene, etc.

Among the azo- and diazo-compounds which can thus be used may be mentioned the following:—diazo-amino-benzene ( $C_6H_5N=N-NH.C_6H_5$ ); diazo-amino-p-toluene; benzene-diazo-amino-p-toluene; formazyl-azo-benzene ( $C_6H_5.N=N)_2C=N.NHC_6H_5$ ; azo-benzene ( $C_6H_5.N=N.C_6H_5$ ); azo-naphthalene (alpha - alpha - derivative); p - amino - azo - benzene,  $C_6H_5.N=N.N.C_6H_4-NH_2$ ; amino-azo-naphthalene; diamino-azo-benzene-hydrochlorid (chrysodin dye); benzene-azo-phenol ( $C_6H_5.N=N.C_6H_4OH$ ); toluene-azo-resorcinol; benzene-azo-a-naphthol, etc. Among the compounds mentioned it will be noted that there are included azo-compounds, amino-azo-compounds, diazo-amino compounds, and oxy-azo compounds or azo phenols. These various compounds may be added either in the form of the free base, or in the form of salts thereof with acid, for example, in the form of the hydrochlorid or sulfate.

Among the various compounds above mentioned, the diazo-amino compounds appear to be the most valuable in promoting the flotation operation, for the reason that they have particularly valuable properties as collecting agents; that is, as agents which cause a very material increase in the recovery of mineral when used in connection with a suitable frothing agent. The amino-azo compounds, and also the oxy-azo compounds, are, in general, less valuable as flotation agents, but are, nevertheless, effective, par-

ticularly as collecting agents. The Sudan dyes, which are also oxy-azo compounds, for example, benzene-azo-b-naphthol, xylene-azo-b-naphthol, benzene-azo-benzene-azo-b-naphthol, a-naphthalene-azo-a-naphthol, the sodium salt of sulfo-benzene-azo-benzene-azo-b-naphthol-sulfonic acid, etc., show a selective action for sulfid minerals, although these dyes proved less advantageous than the amino-azo, diazo-amino and oxy-azo compounds above referred to.

In my companion application, Serial No. 312,249, filed of an even date herewith, I have described and claimed certain improvements in the flotation of minerals and the like, with the aid of hydrazins and hydrazin derivatives. Accordingly, in the present application I do not claim specifically the improvements in which the hydrazins are employed, but I nevertheless intend the present case to be generic to the invention of said companion application, and the more comprehensive claims of the present application to include the process of said companion application. That is, the more comprehensive aspects of the present invention relate to the process in which the flotation operation is carried out with the addition to the ore or mineral pulp of nitrogen compounds containing two nitrogen atoms joined to each other, whether these nitrogen atoms are joined together by a single bond, as in the case of the hydrazin compounds, or by a double bond, as in the case of the azo and diazo compounds; inasmuch as it is new, in so far as I am aware, to carry out the flotation operation with the addition to the ore or mineral pulp of nitrogenous compounds of this character, that is, nitrogenous compounds of the character of azo, diazo, hydrazo, hydrazin, etc., compounds which contain within their molecules the characteristic nitrogen groups of these compounds. The specific claims of the present application are directed to the azo-, and diazo-compounds which contain the doubly bound nitrogen atoms, as distinguished from the hydrazin compounds of said companion application, which have but a single linkage between the two nitrogen atoms.

The azo and diazo compounds can be incorporated with the ore or mineral pulp in any suitable manner, which will insure their uniform incorporation and dissemination throughout the pulp. They may thus be incorporated by grinding in the tube mill in

which the ore is itself ground, or they may be dissolved in an organic solvent therefor and the resulting solution added to the ore pulp, or they may in some cases first be digested in water and the resulting product then added to the ore pulp.

After the azo or diazo compound, either alone or with other flotation agent or agents, has been thoroughly and uniformly distributed throughout the ore or mineral pulp, the resulting mixture is subjected to a flotation operation, as in an ordinary Callow cell, or in apparatus where the air is incorporated in the ore pulp by mechanical agitation.

It is of advantage in many cases to add to the ore pulp a small amount of alkali, sufficient to give the ore pulp a distinct alkaline reaction. The alkali may be added both when the compound is added in the form of the free base, and when it is added in the form of a salt. When a salt of the base is employed, the alkali may act upon it, to a greater or less extent, to set free the free base, but the action of the alkali appears to be an action upon the ore pulp, or upon the mineral constituent, rather than or in addition to its action upon the salt of the compound used, although I do not desire to limit myself by any theoretical explanation of what the action of the added alkali may be in promoting the flotation operation. A similar improvement has been noted both when the alkali has been used with the free base and when used with salts of the base. The alkali may be caustic alkali, such as sodium hydrate, or an alkaline salt, such as sodium carbonate, or even lime or calcium oxide or hydrate can be used.

The amount of the azo or diazo compound added may vary somewhat, and may be as little as one-fifth or one-fourth of a pound per ton of ore; (that is, calculated on the weight of the ore and not of the ore pulp), but larger amounts may, with advantage, be used, particularly where the compound is difficult to uniformly disseminate throughout the ore pulp, and as much as one or one and one-half pounds per ton of ore, or even more, can be used.

The azo and diazo compounds have proven to be of particular value in the flotation of copper sulfid ores having a siliceous gangue and containing their floatable or sulfid copper in the form of a mixture of chalcocite and chalcopyrite, that is, so-called porphyry ores, such as those of the Utah Copper Company. In general, treatment of the ore with alkalis, such as sodium hydrate or lime, gives improved results. In fact, the alkalis themselves seem to have a valuable effect upon the ores in improving the flotation thereof, and the same is true for a number of similar ores. When alkalis are used, it is desirable to give them an appreciable time of contact with the ore pulp before subjecting the lat-

ter to flotation. When possible, it is preferable to add the alkalis in the grinding mill, so that they will be present during the grinding operation.

The following more specific description will further illustrate the invention.

500 parts by weight of the ore, previously crushed to pass a 30 mesh sieve, were placed in the pebble mill, together with the indicated amount of the diazo-amino compound, 250 parts of water, and sodium hydroxid equivalent to two pounds per ton of dry ore, or, in place of the sodium hydroxid, lime in about the same proportion. After the grinding operation, the charge was transferred to a Callow rougher cell and subjected to flotation with the addition of a small fraction of one pound of terpineol per ton of dry ore, or, instead of terpineol, pin oil, or other frothing agent. Terpineol has very little if any collecting power, and functions almost entirely as a frothing agent.

The following are results obtained with certain of the above diazo compounds when used on Utah ore in amounts equal to about one-fifth of a pound per ton of ore:

|                                      | Heads. | Concts. | Ree'y. |    |
|--------------------------------------|--------|---------|--------|----|
| 1. Diazo-amino-benzene .....         | 1.42   | 22.4    | 91.4   | 95 |
| 2. Diazo-amino-p-toluene .....       | 1.42   | 25.7    | 90.6   |    |
| 3. Benzene-diazo-amino-toluene ..... | 1.42   | 24.9    | 91.3   |    |

The diazo-amino compounds are exceedingly powerful collecting agents, even when used in mere traces; for example, as little as one-thirtieth of a pound of diazo-amino-benzene per ton of ore has been found to be sufficient as a collecting agent to give almost maximum results with Utah ore, when used with a small amount of a frothing agent. In general, a frothing agent must be used with these compounds, inasmuch as they have little or no frothing properties themselves, as above pointed out. These compounds are very difficultly soluble solids and are very stable in the air. Continued boiling with water results in their decomposition. They may be dissolved, for flotation purposes, in organic solvents, such as alcohol, anilin, dimethyl-anilin, xylidin, etc. Prolonged heating with other amines may result in chemical changes which reduce the effectiveness of the mixture. Where a solution of one of these compounds in an organic solvent is prepared, it may be added either to the pulp in the grinding mill, or to the ground pulp immediately before flotation. Organic solvents may be properly chosen so as to furnish frothing power to supplement the valuable collecting properties of the diazo and azo compounds. The diazo-amino compounds may also be incorporated in the usual oil mixtures, such as are employed in flotation, and thereby introduced into the pulp, and they will exert a marked influence on the flotation results.

improvement in the flotation results obtained with most, if not all, such oil mixtures. The procedure which I recommend, when it is possible, is to add the reagent in 5 very finely pulverized dry form to the ore pulp in the grinding mill. Frothing agents, such as pine oil, hardwood oil, and various other frothing agents, may be added at the same point, or just previous to flotation, as 10 desired.

The diazo-amino compounds, as above noted, are excellent collecting agents, and this is true as well of the diazo-amino-p-toluene and the benzene diazo-amino-p-toluene, as of the diazo-amino-benzene. The para-amino-azo-benzene and the amino-azo-naphthalene, as well as certain of the oxy-azo compounds, are likewise good collecting agents, but I consider them less valuable than the diazo-amino compounds. 15

Improved results have also been obtained in the flotation of zinc-lead ores, such as those of the Butte and Superior Company. Good results were thus obtained when the 25 diazo-amino compound was ground with the neutral ore pulp, but better results were obtained when copper sulfate and sulfuric acid, in the proportion of one pound of each per ton of dry ore, were also used. A small 30 amount of a suitable frothing agent, as above noted, should also be used.

It is characteristic of the invention that the froth obtained is readily broken up, while a relatively clean concentrate and high 35 recovery can, nevertheless, be obtained. The azo or diazo compound can, moreover, sometimes be recovered, so that it is available for use in the treatment of further amounts of ore, for example, by recovering 40 the circuit water from the concentrates, and even that from the tailings, and returning the same to the process, with resulting economy in the amount required to be added for subsequent operations.

45 The process in which diazo-amino-benzene is used as a collecting agent is claimed specifically in my companion application, Serial No. 312,247, filed of even date here-with.

50 I claim:

1. The method of effecting the concentration of minerals by flotation, which comprises adding to the mineral pulp a small amount of an organic nitrogen compound 55 containing two nitrogen atoms joined to each other, and subjecting the resulting mixture to a flotation operation; substantially as described.

2. The method of effecting the concentration of minerals by flotation, which comprises adding to the mineral pulp a small amount of an organic nitrogen compound containing two nitrogen atoms joined to each other, together with a flotation agent 60 having marked frothing properties, and sub-

jecting the resulting mixture to a flotation operation; substantially as described.

3. The method of effecting the concentration of minerals by flotation, which comprises adding to the mineral pulp a small 70 amount of an organic nitrogen compound containing two nitrogen atoms joined to each other, together with sufficient alkali to give to the ore pulp a distinct alkaline reaction, and subjecting the resulting mixture to 75 a flotation operation; substantially as described.

4. The method of effecting the concentration of minerals by flotation, which comprises adding to the mineral pulp a small 80 amount of an organic nitrogen compound containing two nitrogen atoms joined to each other, together with a flotation agent having marked frothing properties and sufficient alkali to give to the ore pulp a distinct alka- 85 line reaction; and subjecting the resulting mixture to a flotation operation; substantially as described.

5. The method of effecting the concentration of minerals by flotation, which comprises adding to the mineral pulp a small 90 amount of an organic nitrogen compound containing two nitrogen atoms joined to each other by a double bond, and subjecting the resulting mixture to a flotation opera- 95 tion; substantially as described.

6. The method of effecting the concentration of minerals by flotation, which comprises adding to the mineral pulp a small 100 amount of an organic nitrogen compound containing two nitrogen atoms joined to each other by a double bond, together with a flotation agent having marked frothing properties, and subjecting the resulting mixture to a flotation operation; substantially 105 as described.

7. The method of effecting the concentration of minerals by flotation, which comprises adding to the mineral pulp a small 110 amount of an azo compound (*i. e.*, an aromatic compound containing the -N=N- group), and subjecting the resulting mixture to a flotation operation; substantially as described.

8. The method of effecting the concentra- 115 tion of minerals by flotation, which comprises adding to the mineral pulp a small amount of an organic diazo-amino com- 120 pound, and subjecting the resulting mixture to a flotation operation; substantially as de- scribed.

9. The method of effecting the concentra- 125 tion of minerals by flotation, which comprises adding to the mineral pulp a small amount of diazo-amino-toluene, and subject- 130 ing the resulting mixture to a flotation opera- tion; substantially as described.

In testimony whereof I affix my signature.

CLEMENT L. PERKINS.